

## UNITED STATES PATENT OFFICE

2,229,123

## UNHAIRING HIDES AND SKINS

Julius Pfannmuller, North Plainfield, N. J., and  
 Hans Schleich, New Dorp, Staten Island, N. Y.,  
 assignors to Wallerstein Company, Inc., New  
 York, N. Y., a corporation of New York

No Drawing. Application May 2, 1939,  
 Serial No. 271,322

17 Claims. (Cl. 149—2)

This invention relates to a process of treating skins and hides and more particularly to the art of depilating or unhauling skins and hides.

It has long been the common practice to soak 5 skins and hides in a lime or other alkaline bath in order to loosen the hair to such an extent that it can be readily removed mechanically, whether by hand or machine.

One objection to this old process has always 10 been that it was too slow. To meet this objection, it has been customary to add to the lime bath so-called "sharpening" agents such as sodium sulphide, the form of arsenic known as red arsenic and various amines, such as methylamine. 15 While such "sharpening" agents speed up the loosening of the hair, their use is attended with disadvantages of their own. For example, it has been found that most of such "sharpeners" can be used only in limited amounts because too large 20 amounts result in damage to the skins or hides. In fact, even with weak sulphide solutions there is danger of such injury if the bath treatment is prolonged. Moreover, the use of most of these "sharpeners" often if not usually, results in damage 25 to or destruction of the hair. This latter point is of considerable importance because the hair, if it can be reclaimed, is or may be a valuable by-product.

As a solution to the dilemma above outlined, 30 present applicant Julius Pfannmuller has disclosed in a copending application, Serial No. 87,328, a method of treating skins and hides which comprises adding to the lime or other alkaline bath reducing sulphur-oxygen compounds, 35 pounds, of which sodium hydrosulphite is an example. With such a bath, not only is the hair-loosening operation accelerated, as compared to the old lime bath treatment, but there is no damage to the hide or to the hair. Thus, not 40 only is time saved, but the leather, following bating, tanning and other subsequent operations, is of superior quality and the hair can be reclaimed as a by-product.

The sulphur-oxygen compounds in question, 45 and which are hereinafter considered in more detail, are referred to as "accelerators" for convenience and to distinguish them from the so-called "sharpeners" above referred to.

In addition to the coarse long hair, which may 50 be termed the "top" hair, skins and hides have young deep-rooted hair which may be termed "fine" hair. This fine hair presents additional problems in that it is much more difficult to remove than the top hair. On calf skins especially, 55 there is a fine hairy growth or "down" often in-

visible to the eye. If not eliminated, however, such fine hair shows clearly in the leather as soon as the skins are finished. As a result, such leather must be graded lower and, though salable, it cannot bring the price of higher grade leathers. 5 The price difference between two grades of leather is usually large and there may be a differential between the lowest grade and the highest grade, in the same kinds of skins, of several hundred percent.

10 The fine hair can be eliminated by the use of sulphides, such as sodium sulphide, which "burns off" the hair and this procedure is followed in a number of tanneries. But this "burning off" involves loss of the top hair which, as above stated, 15 may be a valuable by-product if it can be reclaimed, and also involves danger of damage to the skins.

In tanneries where the hair is not eliminated by "burning off," the fine hair is usually removed 20 to a greater or less extent as an incident to the operations known as "scudding" and "slating," subsequent to main dehairing. But such removal often causes considerable difficulty and often results in leather requiring low grading. 25 For example, if the hair is not properly loosened, the operator has to press down so much on the skin he is apt to scuff or mechanically damage the same, e. g. by chipping out small areas on the grain. A piece of leather may be perfect except 30 for scuffed or chipped spots or spots of unremoved hairs. But it has to be low graded because it has poor cutting value and shoemakers, for example, will accept as top grade only those skins which have good cutting value. That is, 35 skins which have bad spots will involve a certain loss in cutting because such spots may prevent use of considerable areas.

This problem of hair removal is of relatively 40 little importance if the removal is by hand, as in that case the operator can give each skin a careful and more or less individual treatment. But such hand operations are too costly for the majority of tannery productions. With hair removal by machinery, it is difficult to obtain complete removal of the fine hair, and particularly 45 a uniform removal, without scuffing or damaging the grain of the skin.

As pointed out in the copending application 50 above mentioned, when both an accelerator, such as sodium hydrosulphite, and a sharpener, such as sodium sulphide or red arsenic are added to the bath, the action of the sharpener is greatly enhanced. It follows that when such agents are conjointly used, the requisite period for thorough

hair-loosening is greatly reduced and the danger of damage to the hides by the sulphides consequently reduced. Such a treatment also loosens the fine hair to such an extent that its proper removal involves no great difficulty. Such accelerators, however, do not afford any substantial protection to the hair from the attack of the sharpeners and there is, therefore, danger of damage to the hair. It has been found, for example, that when sodium sulphide ((66% Na<sub>2</sub>S) in amounts above 0.1 percent, based on the soaked weight of hides or skins, is used in a lime or other alkaline bath containing an accelerator, such as sodium hydrosulphite, the hair is attacked to a greater or lesser degree.

The difficulty of properly removing fine hair can be materially lessened, at the same time avoiding the danger of damage to the hair and hide and obviating the necessity of expensive hand-beaming or hand-slating operations, by adding to the lime bath caustic alkali or some substance or substances which will generate caustic alkali therein, for example, soda ash. In the co-pending application referred to, there is disclosed the conjoint use of lime, an accelerator, such as sodium hydrosulphite, and caustic alkali. This solves the problem of removal of fine hair to a certain degree. There is, however, still another problem involved.

If the amount of caustic alkali used is too small, it is still difficult to remove the fine hair. On the other hand, if the amount of caustic alkali used to obtain desired ease of removing fine hair, it may prove to be too great an amount in another respect.

In this connection, and more or less parenthetically, it is to be noted that the various operations involved in the production of leather are more or less inter-related in the sense that while one operation may perform its particular function properly, it may interfere with subsequent operations. For example, a given unhairing bath may properly loosen hair but may so interfere with subsequent bathing, tanning or other operations that good grade leather cannot be obtained.

Returning to the question of too much caustic, when skins or hides are treated in an alkaline bath they become swollen and caustic alkali swells out skins and hides much more than lime alone does. Before the skins can be tanned, they must be "brought down" or "reduced." This is accomplished by an operation known as bathing or puering. Formerly, "puering" was applied to a bath formed from dog manure and "bathing" to a pigeon manure bath or the use of artificial bates containing enzymatic preparations. At present, however, the term "bathing" is more or less commonly used to cover all types of such procedures. The bathing step is carried out both to render the skins soft, supple and flaccid and to bring down or reduce the alkaline swelling. To this end, the operation involves the use of one or more neutralizing agents, the more commonly used agents being ammonium chloride or sulphate.

While some swelling is desired, an excessive swelling makes it next to impossible to bring down the skins or hides properly and is apt to result in a piece of leather of poor, empty break. It follows that in many tanneries and for many kinds of leather, the permissible amount of caustic alkali is subjected to close limitations. Thus, the amount of caustic alkali in the lime bath necessary to obtain thorough and proper action on the fine hair may well be in excess of the limit permissible in respect to the degree of swelling.

It is an object of the present invention to pro-

vide a method of treating skins and hides for the loosening of the hair such that the disadvantages involved in the problems above set forth are avoided.

More particularly it is an object of the invention to provide a hair-loosening treatment such that all the hair, including fine hair, can be removed properly and without undue difficulty and without resort to hand removal and, at the same time, such that there is no substantial damage or injury to hide or hair; such that excessive swelling of the skins or hides is avoided; and such that proper leather of good grade can be subsequently obtained.

We have discovered that when hides and skins are subjected, for example, to the action of lime, sodium sulphide and sodium hydrosulphite under proper conditions and in a particular sequence, a new and unexpected result is obtained as compared to any of the procedures above outlined and more particularly as compared to the action of a bath containing lime, sulphide and hydrosulphite simultaneously. By such treatment we attain a substantial improvement over the procedures above outlined.

In carrying out the invention, and citing the materials specified by way of example, we first subject the hides or skins to the action of a sodium sulphide solution in the absence of lime or other alkaline material. We then subject such hides or skins to the action of a lime bath containing sodium hydrosulphite.

To this end, we first immerse the hides or skins in an aqueous bath containing sodium sulphide. In tannery practice, it is the usual custom to wash and soak skins and hides prior to any treatment with chemicals. The sodium sulphide may be added to the soak water at any time after a short preliminary wash or the skins or hides may be subjected to the sulphide solution after the soaking operation.

While the time of treatment in the sulphide bath may vary, treatments of from one-half hour to twenty four hours have been found to give satisfactory results. Generally speaking, the shorter the soaking period prior to the sulphide treatment the longer should the skins or hides remain in the sulphide solution. However, even with a long soaking, a relatively long sulphide treatment may be used.

The sulphide treatment may be conveniently, but not necessarily, carried out in the paddle ordinarily used in the leather industry, the washed skins being placed therein and the sulphide added to the water. The relative amount of water used may vary but a skin-to-water ratio of about 1 to 4, based on soaked or wet salted skin weight, has been found to give satisfactory results. For dry skins, considerably more water will ordinarily be required.

The bath temperature may be in what may be termed the normal range i. e. from 55° to 70° F. or somewhat higher. It is considered inadvisable to use temperatures above 100° F. In the event of an abnormal drop in room temperature during the process, it may be advisable to adjust the bath temperatures since lower temperatures slow up the process.

The relative amount of sodium sulphide used may vary. In this connection, we have discovered that the available range depends, at least in part, on the pH value of the sulphide solution and that the range can be widened by properly controlling such pH value.

Regardless of pH value, the least amount of

sodium sulphide that is sufficient to obtain what are now considered practically effective results, is about  $\frac{1}{2}$  pound concentrated sodium sulphide (66% Na<sub>2</sub>S) per 1000 pounds of skins or hides, 5 figured on soaked weight. An amount between that minimum up to about 5 pounds of such sodium sulphide per 1000 pounds of skins or hides gives satisfactory results and within that range it is normally unnecessary to pay any particular 10 attention to the pH value. If higher proportions are used, the hair is more or less attacked unless the pH value of the bath is properly adjusted. If, for any reason, it is desired to use a higher proportion of sodium sulphide, the danger of 15 damage to the hair can be avoided by adjusting the alkaline reaction of the solution to a pH value below 11.7. We have found that what are now considered the best results are obtained if the pH value is adjusted to around 10.6 or lower. 20

If adjustment of the pH value is indicated, this may be effected by means of any suitable agent for reducing the alkalinity. Examples of such agents are sulphuric, muriatic, boric or organic acids; sodium bicarbonate or borate; or other 25 acid salts or salts of a weak base such as ammonium chloride; or organic amines.

If and when the pH value is thus adjusted, the relative amount of sodium sulphide used may be safely increased up to 10 pounds per 1000 30 pounds of skins or hides. Even a somewhat larger proportion of sodium sulphide may be used without serious damage to the hair or skins but it is our present belief that with amounts above the maximum mentioned there is no such increase 35 in effectiveness as to warrant such increase in proportions.

After the sulphide treatment above described, the sulphide solution is drained off and the skins or hides may, if desired, be slightly washed.

Then the skins are subjected to the action of a lime bath to which is added an accelerator such, 40 for example, as sodium hydrosulphite (Na<sub>2</sub>S<sub>2</sub>O<sub>4</sub>). In this connection, we are aware that there is some difference of opinion among chemists as to the use of the term "hydrosulphite" for salts of 45 the acid H<sub>2</sub>S<sub>2</sub>O<sub>4</sub>. There appears to be a recent tendency, more particularly in some foreign countries, to designate such salts as "hyposulphites." In view, however, of the fact that the term "hyposulphites" has long been used in this and other 50 countries to designate salts of thiosulphuric acid (H<sub>2</sub>S<sub>2</sub>O<sub>3</sub>), more properly called thio-sulphates, we prefer to use the term "hyposulphites" for salts of the acid H<sub>2</sub>S<sub>2</sub>O<sub>4</sub>.

Assuming that the skins or hides have been 55 subjected to the sulphide treatment in a paddle, the most convenient procedure is to replace the sulphide liquor with water and then mix in the lime and sodium hydrosulphite. For this bath, we have found it advisable to have the bath temperature above approximately 60° F., say from 60 70° to 86° F.

The relative amount of lime used may vary 65 within a considerable range. Ordinarily, amounts between about 100 pounds and 250 pounds per 1000 pounds of skins or hides, based on soaked weight, give satisfactory results but occasionally a somewhat higher proportion is desirable.

The relative amount of sodium hydrosulphite 70 may also vary. We have found that from 4 pounds to 6 pounds per 1000 pounds of skins or hides (soaked weight) gives satisfactory results. Smaller proportions may be used but will be less effective. Larger proportions may also be used 75 but amounts materially greater than those indi-

cated do not appear to effect any substantial change in the results, and, hence, are unnecessary.

While the duration of treatment in the lime-hydrosulphite bath may vary, we have found that a treatment of from 2 to 4 days, measured from 5 the time the lime is added, gives satisfactory results, the hair, including fine hair, being in such a thoroughly loosened condition as to be readily and properly removable by normal tannery procedure. In this connection it should be noted 10 that the hair will probably be thoroughly loosened in considerably less than 4 days. As previously suggested, however, the various operations involved in the production of leather are interrelated. Most tanneries consider that the duration 15 of the lime or other alkaline treatment controls, to a considerable extent, the texture of the final leather. It follows that the duration of treatment in the lime bath does not depend on the hair loosening factor alone and a longer treatment than required for proper hair loosening may 20 be desirable for other reasons.

Skins and hides treated according to the invention as so far described will have an alkaline swelling well below any degree of swelling that 25 is considered excessive in the sense hereinabove referred to. In fact, in many cases, there will not be as much swelling as tanners desire. In such case, the degree of swelling may be increased by adding to the lime-hydrosulphite bath a caustic 30 alkali. While the amount may vary, we have found that from .05 percent to 5.0 percent, based on soaked or wet salted skin weight gives satisfactory results, the proportion used depending largely on the degree of swelling desired. That 35 is, the more swelling desired, the greater the proportion of caustic used. In referring to the addition of a caustic alkali, it is to be understood that we include addition of caustic alkali as such or the addition of any compound that will generate 40 caustic alkali in the lime bath, for example, soda ash or sodium sulphite.

Instead of using sodium sulphide in the first bath, other alkaline sulphides may be used.

Instead of using sodium hydrosulphite, other 45 accelerators may be used. For the purposes of the present application, "accelerators" are to be understood to mean reducing sulphur-oxygen combinations, characterized by being relatively stable in the dry state and having a substantially 50 greater reducing power in solution than that of the sulphates, sulphites, sulphides or thio-sulphates. Such combinations include compounds of the class of hydrosulphites and sulphoxylates, e. g. sodium, calcium, magnesium and zinc hydrosulphites and sulphoxylates, and corresponding 55 organic compounds of sulphur and oxygen, such as the aldehyde and ketone derivatives of the hydrosulphites and sulphoxylates. Further examples are sodium, calcium, or magnesium formaldehyde sulphoxylate; zinc calcium hydrosulphite; sodium, calcium, magnesium or zinc formaldehyde sulphoxylate or hydrosulphite and other hydrosulphites and sulphoxylates of sodium, calcium, magnesium and zinc. In short, all sulphuric or disulphuric acid derivatives whether of inorganic or organic origin, aromatic or aliphatic, 60 may be used.

Instead of lime, or in conjunction with lime, other alkaline materials such, for example, as 65 caustic soda or soda ash, may be used.

With the treatment described, the hair, including fine hair, is so thoroughly loosened it can readily be removed by normal tannery processes 70 and without the necessity of recourse to removal 75

by hand. At the same time there is no substantial damage or injury to the hair and, thus, the hair can be reclaimed as a by-product. Nor is there any substantial damage or injury to the 5 hides and, thus, it is possible to produce proper leather of high grade. Moreover, these beneficial results are obtained without entailing excessive alkaline swelling of the skins or hides.

It has been proposed in a United States patent 10 to treat skins and hides, first in a sulphide solution of an alkalinity represented by a pH of 11.8 to 12.2 and thereafter to the action of a lime bath. It is stated in such patent that the procedure referred to avoids damage or injury to hide or 15 hair. Whether or not this is true, is a point not here involved. In any event, we have found that with the procedure proposed in such patent the fine hair is often, if not usually, difficult to remove. Moreover, we have found that with the 20 pH values prescribed by the patentee as critical and with the proportions of sulphides prescribed by him, the hair is definitely attacked and damaged if, after the sulphide treatment, the skins or hides are subjected to a bath such as we here propose, namely, a bath containing lime and an 25 accelerator, such as sodium hydrosulphite.

The following more detailed procedures are given by way of example, such procedures having been found to give satisfactory results.

30 In each case the hair, including the fine hair, was readily removed. If any fine hair was left after the removal of the main hair, it was removed without difficulty as an incident to scudding. The top hair was of good quality and could be re- 35 claimed as a by-product. The leather, following bating, pickling, tanning, etc. was of excellent quality and good grade.

Where the addition of chemicals is specified, sufficient agitation to obtain a proper mix is to 40 be understood. "Lime" means hydrated lime throughout.

#### Example I

1000 pounds calfskins (salted weight) were washed in a drum for about 2 hours and then 45 hair fleshed. The skins were then transferred to a paddle containing sufficient water to give a skin-to-water ratio of about 1:4. To this water had been added 3 1/4 pounds fused sodium sulphide (66% Na<sub>2</sub>S). The skins were paddled for 30 minutes and allowed to stand in the sulphide bath for 17 hours.

The sulphide solution was drained off and replaced by water at about 78° F. 100 pounds of lime were then added. After a short paddling, 55 there was added 5 pounds sodium hydrosulphite. After 20 hours, 2.5 pounds soda ash were added and the paddle turned a short time.

After a total of 3 days in the lime bath the skins were removed and unhaired on the usual unha- 60 ring machine.

#### Example II

1000 pounds calfskins were soaked overnight and put in a paddle having sufficient water to give 65 a skin-to-water ratio of 1:4.5. Then there was added 4 pounds sodium bicarbonate and, after 10 minutes, 6 pounds sodium sulphide (66% Na<sub>2</sub>S).

The skins were kept in this bath for 17 hours. The pH of the soak liquor at end of soaking was 70 9.5.

The sulphide solution was drained off and replaced by water at 80° F. Then there was added 100 pounds lime and, after 20 minutes, 6 pounds sodium hydrosulphite. After 2 days in the lime 75 bath the skins were unhaired.

#### Example III

1000 pounds goatskins, dry weight, were soaked for one day and put in a paddle containing about 7000 pounds water at about 75° F. Then there was added, in the batches, a total of 8 pounds crystallized sodium sulphide (33% Na<sub>2</sub>S approx.). The skins were paddled for 1 1/2 hours. The pH shortly after the first addition was 8.7; after the second addition and at end of paddling, 9.3. The skins were kept in this bath over night.

Next morning the pH of the sulphide liquor was 8.5. The sulphide liquor was drained off and replaced by water at 80° F. There was then added 300 pounds lime and 3 pounds sodium hydro- 15 sulphite. After paddling for one hour and a rest period of 2 hours, there was added 12 pounds soda ash and 7 pounds more sodium hydrosulphite.

After 72 hours the liquor was drained off. The skins were kept overnight in cold water and then removed and dehaired.

#### Example IV

2000 pounds salted calfskins were soaked for 17 hours and put in a paddle containing sufficient water to give a skin-to-water ratio of 1:4.5. Then there was added 8 pounds sodium bicarbonate and, after 10 minutes 12 pounds sodium sulphite (66% Na<sub>2</sub>S). The skins were left in this bath 3 hours, after which time the pH was found to 30 be 10.0.

The sulphide solution was replaced by water at 80° F. To this there was added 200 pounds lime, and, after 20 minutes, 12 pounds sodium hydrosulphite. The skins were left in this bath 35 overnight. Next day there was added 5 pounds soda ash. After a total of 3 days following addition of the lime the skins were removed and unhaired.

#### Example V

2000 pounds calfskins were soaked for 16 hours and put in a paddle containing sufficient water to give a skin-to-water ratio of 1:4.5. Then there was added 2.5 pounds sodium sulphide (66% Na<sub>2</sub>S). The skins were left in this sulphide bath for 4 hours.

The sulphide solution was replaced by water at 78° F. To this was added 200 pounds lime and, after 20 minutes, 12 pounds sodium hydrosulphite. After 24 hours there was added 10 pounds soda 50 ash.

After remaining in the lime bath 3 days the skins were removed and unhaired.

What is claimed is:

1. The method of loosening the hair of skins and 55 hides which comprises subjecting the skins or hides to the action of an aqueous bath to which has been added an alkaline sulphide and which is substantially free of any other alkaline material, and thereafter subjecting the skins or hides 60 to the action of an aqueous bath to which has been added an alkaline material and a material selected from the group consisting of hydrosulphites, sulphoxylates and their aldehyde and ketone derivatives.

2. The method of loosening the hair of skins and 70 hides which comprises subjecting the skins or hides to the action of an aqueous bath to which has been added an alkaline sulphide and which is substantially free of any other alkaline material, and thereafter subjecting the skins or hides 75 to the action of an aqueous bath to which has been added lime and a material selected from the group consisting of hydrosulphites, sulphoxylates and their aldehyde and ketone derivatives.

3. The method of loosening the hair of skins and hides which comprises subjecting the skins or hides to the action of an aqueous bath to which has been added an alkaline sulphide and which is substantially free of any other alkaline material, and thereafter subjecting the skins or hides to the action of an aqueous bath to which has been added an alkaline material and a hydrosulphite. 5
4. The method of loosening the hair of skins and hides which comprises subjecting the skins or hides to the action of an aqueous bath to which has been added an alkaline sulphide and which is substantially free of any other alkaline material, and thereafter subjecting the skins or hides to the action of an aqueous bath containing lime and a hydrosulphite. 10
5. The method of loosening the hair of skins and hides which comprises subjecting the skins or hides to the action of an aqueous bath to which has been added sodium sulphide and which is substantially free of any other alkaline material, and thereafter subjecting the skins or hides to the action of an aqueous bath containing an alkaline material and sodium hydrosulphite. 15
6. The method of loosening the hair of skins and hides which comprises subjecting the skins or hides to the action of an aqueous bath to which has been added sodium sulphide and which is substantially free of any other alkaline material, and thereafter subjecting the skins or hides to the action of an aqueous bath containing lime and sodium hydrosulphite. 20
7. The method of loosening the hair of skins and hides which comprises subjecting the skins or hides to the action of an aqueous bath to which has been added an alkaline sulphide and which is substantially free of any other alkaline material, adjusting the alkaline reaction of the bath to a pH value below 11.7, and thereafter subjecting the skins or hides to the action of an aqueous bath to which has been added an alkaline material and a material selected from the group consisting of hydrosulphites, sulphoxylates and their aldehyde and ketone derivatives. 25
8. The method of loosening the hair of skins and hides which comprises subjecting the skins or hides to the action of an aqueous bath to which has been added an alkaline sulphide and which is substantially free of any other alkaline material, adjusting the alkaline reaction of the bath to a pH value below 11.7, and thereafter subjecting the skins or hides to the action of an aqueous bath to which has been added lime and a material selected from the group consisting of hydrosulphites, sulphoxylates and their aldehyde and ketone derivatives. 30
9. The method of loosening the hair of skins and hides which comprises subjecting the skins or hides to the action of an aqueous bath to which has been added sodium sulphide (66% Na<sub>2</sub>S) in an amount between approximately 1/2 pound and approximately 5 pounds per 1000 pounds of skins or hides, figured on soaked weight, and which is substantially free of other alkaline material, and thereafter subjecting the skins or hides to the action of an aqueous bath to which has been added lime and a material selected from the group consisting of hydrosulphites, sulphoxylates and their aldehyde and ketone derivatives. 35
10. The method of loosening the hair of skins and hides which comprises subjecting the skins or hides to the action of an aqueous bath to which has been added sodium sulphide (66% Na<sub>2</sub>S) in an amount between approximately 1/2 pound and approximately 5 pounds per 1000 pounds of skins 40
- or hides, figured on soaked weight, and which is substantially free of other alkaline material, and subjecting the skins or hides to the action of an aqueous bath to which has been added lime and sodium hydrosulphite. 5
11. The method of loosening the hair of skins and hides which comprises subjecting the skins or hides to the action of an aqueous bath to which has been added sodium sulphide (66% Na<sub>2</sub>S) in an amount in excess of approximately 5 pounds per 1000 pounds of skins or hides, figured on soaked weight, and which is substantially free of other alkaline material, adjusting the alkaline reaction of the bath to a pH value below 11.7, and thereafter subjecting the skins or hides to the action of an aqueous bath to which has been added an alkaline material and a material selected from the group consisting of hydrosulphites, sulphoxylates and their aldehyde and ketone derivatives. 10
12. The method of loosening the hair of skins and hides which comprises subjecting the skins or hides to the action of an aqueous bath to which has been added sodium sulphide (66% Na<sub>2</sub>S) in an amount in excess of approximately 5 pounds per 1000 pounds of skins or hides, figured on soaked weight, and which is substantially free of other alkaline material, adjusting the alkaline reaction of the bath to a pH value below 11.7, and subjecting the skins or hides to the action of an aqueous bath to which has been added lime and sodium hydrosulphite. 15
13. The method of loosening the hair of skins and hides which comprises subjecting the skins or hides to the action of an aqueous bath to which has been added an alkaline sulphide and which is substantially free of any other alkaline material, and thereafter subjecting the skins or hides to the action of an aqueous bath to which has been added lime and sodium hydrosulphite, the latter being added in an amount from about 4 pounds to about 6 pounds per 1000 pounds of skins or hides, figured on soaked weight. 20
14. The method of loosening the hair of skins and hides which comprises subjecting the skins or hides to the action of an aqueous bath to which has been added an alkaline sulphide and which is substantially free of any other alkaline material, and thereafter subjecting the skins or hides to the action of an aqueous bath to which has been added lime and a material selected from the group consisting of hydrosulphites, sulphoxylates and their aldehyde and ketone derivatives, said second bath also containing a caustic alkali. 25
15. The method of loosening the hair of skins and hides which comprises soaking the skins or hides in water, adding to the soak water an alkaline sulphide, leaving the skins or hides in such bath for from 1/2 to 24 hours, replacing said bath with water, adding an alkaline material and a material selected from the group consisting of hydrosulphites, sulphoxylates and their aldehyde and ketone derivatives, and leaving the skins or hides in said second bath for from 2 to 4 days. 30
16. The method of loosening the hair of skins and hides which comprises subjecting the skins or hides to the action of an aqueous bath, at normal temperature, to which has been added an alkaline sulphide and which is substantially free of other alkaline material, and thereafter subjecting the skins or hides to the action of a warm water bath to which has been added an alkaline material and a material selected from the group consisting of hydrosulphites, sulphoxylates and their aldehyde and ketone derivatives. 35

17. The method of loosening the hair of skins and hides which comprises subjecting the skins or hides to the action of an aqueous bath to which has been added an alkaline sulphide and which is substantially free of any other alkaline material, thereafter subjecting the skins or hides to the action of an aqueous bath to which has been

added lime and sodium hydrosulphite, and controlling the degree of swelling of the skins or hides by adding to said second bath suitable amounts of a caustic alkali.

JULIUS PFANNMULLER.  
HANS SCHLEICH.

CERTIFICATE OF CORRECTION.

Patent No. 2,229,123.

January 21, 1941.

JULIUS PFANNMULLER, ET AL.

It is hereby certified that error appears in the printed specification of the above numbered patent requiring correction as follows: Page 3, first column, line 53, for " "hyposulphites" " read --"hydrosulphites"--; and that the said Letters Patent should be read with this correction therein that the same may conform to the record of the case in the Patent Office.

Signed and sealed this 18th day of February, A. D. 1941.

(Seal)

Henry Van Arsdale,  
Acting Commissioner of Patents.